

## UNITED STATES PATENT OFFICE

2,161,254

## SILVER-MAGNESIUM CONTACT

Frans R. Hensel and Kenneth L. Emmert, Indianapolis, Ind., assignors to P. R. Mallory & Co., Inc., Indianapolis, Ind., a corporation of Delaware

No Drawing. Application March 18, 1938,  
Serial No. 242,727

4 Claims. (CL 200—166)

This invention relates to electric contacts.

The present invention constitutes an improvement on the invention set forth in co-pending application Serial #223,506.

5 An object of the invention is to improve the characteristics of the electric contact elements containing silver.

Another object of the invention is to provide a silver base contact material, which will retain 10 a very low contact resistance.

15 A still further object is to provide a new contact material which can be used under severe electrical loads, without welding or sticking.

It is a further object of the invention to provide a contact, capable of operating on high frequency and heavy current values, without objectionable metal transfer.

20 Other objects of the invention will be apparent from the following description, taken in connection with the appended claims.

25 The present invention comprises a combination of elements, methods of manufacture and the products thereof, brought out and exemplified in the disclosure hereinafter set forth, the scope of the invention being indicated in the appended claims.

While a preferred embodiment of the invention is described herein, it is contemplated that a considerable variation may be made in the method of procedure, and the combination of 30 elements, without departing from the spirit of the invention.

The present invention comprises an improvement in silver base electric contact elements.

According to the invention, the contacts are 35 improved by the addition of small percentages of magnesium.

The contacts are composed of silver and magnesium, the ingredients being present in the following proportions:

40 Magnesium \_\_\_\_\_ per cent 2 to 3.8  
Silver \_\_\_\_\_ Balance

We have discovered that contact alloys of 2 to 3.8% magnesium exhibit a surprising increase in 45 current carrying or interrupting capacity. The greatest current capacity appears to be achieved with alloys containing 3 to 3.6% magnesium. In comparative tests contacts of this composition withstood 27 amperes without welding together 50 while interrupting a 12 volt D. C. circuit at a frequency of 470 cycles per second. Contacts of fine silver, similarly tested had a critical current value of 12 amperes and those of coin silver a current value of 11 amperes under the same 55 conditions.

It is also found that the amount of material

transfer from contact to contact during operation is very low with this composition.

The electrical conductivity of the alloy likewise decreases rapidly above the range of compositions described.

5 The contact resistance of the present alloy is as low as that of fine silver and some compositions are even lower. The alloy has a definite advantage that the contact resistance values are not erratic, but very constant. It is often 10 found with other contact alloys that in service, a high contact resistance will be built up after a short period of operation, and if the contacts continue in operation, the contact resistance might drop down again to lower values, and vary 15 as much as 10 milliohms. Such is also the case with fine silver.

An outstanding advantage of the alloys with the limited range of compositions, as given above, is that materials of this type can be easily swaged 20 and drawn into the form of wires or rolled into the form of sheet, from which contacts may be prepared by a punching operation, screw machine operation, cold heading, and the like. The alloy has an electrical conductivity of 25 to 30% I. A. C. S. and similarly high thermal conductivity which is important, because it will prevent 25 over-heating of the contacts.

The new silver-magnesium alloy can readily be prepared in the form of contact bi-metals, in 30 which one side consists of a base metal and the other side of the silver-magnesium alloy.

While the present invention as to its objects and advantages has been described herein, as carried out in specific embodiments thereof, it 35 is not desired to be limited thereby, but it is intended to cover the invention broadly, within the spirit and scope of the appended claims.

What is claimed is:

1. An electric contact formed of an alloy of 2 to 3.8% magnesium and the balance silver. 40

2. An electric contact formed of an alloy of 3 to 3.6% magnesium and the balance silver.

3. An electric contact formed of an alloy of 2 to 3.8% magnesium and the balance substantially 45 all silver, characterized by a high current carrying and interrupting capacity, low contact resistance and low material transfer tendency during contact operation.

4. An electric contact formed of an alloy of 3 to 3.6% magnesium and the balance substantially 50 all silver, characterized by a critical current interrupting capacity during contact operation greater than twice that of fine silver.

FRANZ R. HENSEL, 55  
KENNETH L. EMMERT.